

## UNITED STATES PATENT OFFICE

VANDERVEER VOORHEES, OF HAMMOND, INDIANA, ASSIGNOR TO STANDARD OIL COMPANY, OF WHITING, INDIANA, A CORPORATION OF INDIANA

## ANTIKNOCK GASOLINE

No Drawing.

Application filed December 15, 1928. Serial No. 326,414.

This invention relates to anti-knock gasoline of the vapor phase type, which results from the cracking of petroleum oils at high temperatures and in the vapor phase, where-  
5 by anti-knock qualities which are, for exam-  
ple, equivalent to those of a straight-run mid-  
continent gasoline containing from about 1.2  
to 4 ccs. tetraethyl lead per gallon are ob-  
tained.

10 In order more fully to define the gasoline to which the present invention relates, it may be stated that such a gasoline with 425° F. end point, has an A. P. I. gravity of about 49 to 55°, an unsaturated content as determined  
15 by sulfuric acid absorption and polymeriza-  
tion exceeding 40% and usually above 45%, and an oxygen absorption induction period of less than 125 minutes when subjected to test under the conditions set forth in co-pend-  
20 ing application, Serial No. 211,554, filed Au-  
gust 8, 1927, by T. H. Rogers and the present inventor.

The anti-knock qualities of such gasoline vary within wide limits, depending primarily  
25 upon the conditions of manufacture and, also, the crude oil from which it is derived.

It has now been discovered that gasoline of this type possesses the serious disadvantage that during the course of time, the anti-knock  
30 quality seriously deteriorates. Average measure-  
ments made on a large number of samples of vapor phase anti-knock gasoline show conclusively that the anti-knock quality deteriorates progressively with time of storage.  
35 Thus, such gasolines, having an average anti-  
knock of about 1 to 3 ccs. of tetraethyl lead per gallon of a standard gasoline, suffered a deterioration of anti-knock quality of about 25% in two months, 50% in five months and  
40 75% in nine months. At the end of twelve months, the anti-knock value was approxi-  
mately zero for many samples.

This deterioration of anti-knock quality raises a serious economic problem since it is  
45 frequently impossible to avoid the storage of gasoline in bulk for substantial periods of time. The loss involved amounts to substan-  
tial sums of money since the anti-knock qual-  
ity is of substantial value, representing a pre-  
50 mium of several cents per gallon.

I have now discovered that vapor phase cracked gasoline, which has deteriorated with respect to anti-knock qualities, may be restored substantially to its original degree of anti-knock effectiveness by redistillation to 55 end point, leaving a small quantity of residue, of the order of 1%. Average results from a large number of experiments indicated that such gasolines which have substantially completely deteriorated with respect to anti-  
knock qualities are restored in this way, to 60 the extent of about 90% of their original anti-knock value. Gasoline which has deteriorated to a lesser extent is restored even closer to its original effectiveness. 65

I claim:

1. The method of regenerating the anti-  
knock qualities of vapor phase cracked gaso-  
line having a substantial initial anti-knock  
effectiveness equivalent to those of straight 70  
run mid-continent gasoline containing up-  
ward of one to two cubic centimeters of lead  
tetra ethyl per gallon, which gasoline has de-  
teriorated in anti-knock effectiveness during  
storage for a substantial period of time, which 75  
consists in subjecting said gasoline to a non-  
cracking redistillation, leaving a small quan-  
tity of residue, of the order of one percent.

2. The method of regenerating the anti-  
knock qualities of vapor phase cracked gaso-  
line having a substantial initial anti-knock  
effectiveness equivalent to those of straight 80  
run mid-continent gasoline containing up-  
ward of one to two cubic centimeters of lead  
tetra ethyl per gallon, which gasoline has de-  
teriorated in anti-knock effectiveness during  
storage for a substantial period of time, which 85  
consists in subjecting said gasoline to a non-  
cracking redistillation, leaving a residue  
due of at least one percent. 90

In witness whereof, I have hereunto set my  
hand this 11th day of December, 1928.

VANDERVEER VOORHEES.